

# United States Patent Office

3,578,441  
Patented May 11, 1971

## 1

3,578,441  
ALLOY

Otto Knotek, Lausanne, Switzerland, assignor to Eutectic Corporation, Flushing, N.Y.  
No Drawing. Filed Nov. 4, 1968, Ser. No. 773,285  
Int. Cl. C22c 19/02

U.S. Cl. 75—171

4 Claims

### ABSTRACT OF THE DISCLOSURE

This invention relates to an alloy capable of being polished to a mirrorlike finish. The alloy is very hard having a hardness of up to 1200 on the Vickers scale and comprises a nickel base with high boron content, up to nine percent by weight, with chromium.

There has been a need in the art for an alloy that would provide a tough, wear resistant hard surface that could be polished to bright mirrorlike finish, to take the place of some of the plated alloys (such as chrome plating) which cannot maintain their high finish during hard service.

The general object of the present invention is to provide an alloy that can be polished to an extremely high smooth and lustrous finish.

The alloy of the present invention comprises the alloying of elemental nickel with chromium and boron. It was found that with high boron additions, up to nine percent by weight, a boron, chrome, nickel trinary alloy can be formed with a high incidence of nickel borides and chrome borides. This alloy having a high degree of nickel borides and chrome borides is very hard, up to 1200 on the Vickers scale and the boride integration permit a highly lustrous mirrorlike finish. This alloy, it has been found, has remarkably reduced voids.

The alloy of the present invention has the following alloy composition in the weight percentages indicated:

| Element  | Range, weight percent | Preferred range, weight percent |
|----------|-----------------------|---------------------------------|
| Boron    | 6 to 9                | 6.7 to 8.3                      |
| Chromium | 3.3 to 7.3            | 4.3 to 6.5                      |
| Nickel   | Balance essentially   | Balance essentially             |

## 2

A typical example of an alloy of the present invention is one with a nominal composition of 7% boron, 6% chromium and balance essentially nickel (with the usual minor impurities).

5 It will therefore be understood by those skilled in the art that an alloy has been provided with a hard lustrous finish. The alloy can be manufactured by any number of the processes known in the art such as by casting and later grinding and polishing to a highly lustrous finish.

10 I claim:

1. An alloy consisting essentially of the following composition in the weight percentages indicated:

| Element: | Weight percent      |
|----------|---------------------|
| Boron    | 6 to 9              |
| Chromium | 3.3 to 7.3          |
| Nickel   | Balance essentially |

2. The alloy of claim 1 wherein said alloy composition is of the following composition in the indicated weight percentages:

| Element: | Weight percent      |
|----------|---------------------|
| Boron    | 6.7 to 8.3          |
| Chromium | 4.3 to 6.5          |
| Nickel   | Balance essentially |

3. The alloy of claim 2 that can be polished to a lustrous finish.

30 4. The alloy of claim 3 with a hardness of up to 1200 on the Vickers scale.

### References Cited

#### UNITED STATES PATENTS

|              |        |         |        |
|--------------|--------|---------|--------|
| 35 2,875,043 | 2/1959 | Tour    | 75—171 |
| 2,936,229    | 5/1960 | Shepard | 75—171 |

40 RICHARD O. DEAN, Primary Examiner